

J. E. LAPPEN:  
PROCESS OF MAKING PAPER STOCK FROM CEREAL STRAW,  
APPLICATION FILED APR. 21, 1916.

1,236,723.

Patented Aug. 14, 1917.

Fig. 1



Fig. 2



Inventor:

James E. Lappen  
by: Bothrop & Johnson  
Attnys.

# UNITED STATES PATENT OFFICE.

JAMES E. LAPPEN, OF WINONA, MINNESOTA, ASSIGNOR TO WINONA PULP & PAPER COMPANY, OF WINONA, MINNESOTA, A CORPORATION.

## PROCESS OF MAKING PAPER-STOCK FROM CEREAL STRAW.

1,236,723.

Specification of Letters Patent. Patented Aug. 14, 1917.

Application filed April 21, 1916. Serial No. 92,607.

To all whom it may concern:

Be it known that I, JAMES E. LAPPEN, a citizen of the United States, residing at Winona, in the county of Winona and State 5 of Minnesota, have invented certain new and useful Improvements in Processes of Making Paper-Stock from Cereal Straw, of which the following is a specification.

My invention relates to improvements in 10 the art of making paper stock, including so-called "half-stock," from cereal straw, such as wheat, oats, barley, and the like. In such straw the fibers are comparatively short and are bound together by the natural gums of 15 the plant with varying degrees of strength in the different parts of the straw,—the fibers in the stalk, for instance, holding together more tenaciously than those in the chaff or the leaves; and with the straw as it 20 is taken from the field there is always more or less weed and other foreign matter, so that the length and severity of the treatment necessary to remove the gums and 25 separate the fibers in the different parts of the material will naturally vary. It is important therefore that the process shall not be such as to destroy the fibers in the weaker parts while the more refractory parts are being reduced.

30 It has been customary heretofore to cook the straw in open vats or rotary digesters, under no pressure other than atmospheric pressure, until the gummy constituents which bind the straw fibers together have 35 been loosened up and the coloring matter released, and then to pour off the gummy liquor, which has become brown from taking up this coloring matter, and empty the vessel of the mushy cooked mass. But notwithstanding 40 that the liquor is thus poured off some of it will always remain in the mass and not only give it color but form hard and lumpy parts, owing to the reuniting of the gum with the fibers when the 45 mass gets cold or dry. It is therefore customary, after the mass has been cooked, to wash it in order more completely to remove the coloring matter and gummy constituents, and then to beat it in a beating machine 50 in order to break up the hard and lumpy parts so formed. But even when the stock is passed through the washing and beating apparatus, it will produce a paper

which has hard slivers and particles of browner color embedded therein, because of 55 the incomplete removal of the gums and separation of the fibers. Besides, the washing process is objectionable because a considerable amount of the stock will be washed away, and the beating is undesirable because it breaks up the fibers. 60

Sometimes also the fibrous mass has been treated at some stage of the process with alkalis or other chemicals in the effort to remove the gums. But with a stock of straw 65 such as above described wherein the fibers in the different parts of the straw are bound together with varying degrees of strength, the fibers in the weaker portions of the straw, such as the chaff and leaves, will be 70 apt to be destroyed by the treatment before the fibers in the stronger parts, such as the stalks, have been fully degummed and separated.

It is the object of this process to improve 75 the method of treating the straw by thoroughly removing the coloring matter and the gummy constituents that bind the fibers together while the cooked mass is still warm and in the digester and without the use of 80 chemicals, so as to prevent the gums and coloring matter from remaining in the wet mass and reuniting with the fibers after they have once been softened and separated therefrom, thereby making unnecessary the 85 subsequent washing and chemical treatment with its resultant loss of stock and the treating of the stock in a beating machine with the undesirable breaking up of the long fibers which give strength to the paper made 90 from it, and avoiding the waste of fiber inherent in the chemical treatment of the stock.

In carrying out my improved process I first cook the straw under pressure until the gummy constituents and coloring matter have become loosened up and washed out and then drive out the brown, gummy liquor by forcing water through the fibrous mass while the same is still heated and under 100 pressure. While the process is not dependent upon the particular sort of apparatus used in carrying it out, yet I have found the apparatus illustrated in the accompanying drawings particularly suitable for the 105 purpose.

## In the drawings,

Figure 1 is a view partly in side elevation, and partly in vertical section, of the digester in which I carry out the process; and

5 Fig. 2 is a top view of the same.

In the drawings, A represents the digester or boiler in which the straw is to be treated. Leading into the bottom of this digester at diametrically opposite points are two pipes 10 2, which are branches of a pipe 3 through which water and steam or either water or steam can be introduced into the digester, the water being supplied to the pipe 3 through a valved water supply pipe 4, and 15 the steam through a valved steam pipe 5, both of which pipes lead into a common union 6 in the pipe 3. In the pipes 4 and 5 are valves 7 and 8, respectively, whereby to control the supply of water and 20 steam to the pipe 3, which leads to the digester.

At the top of the digester is a valved outlet pipe 9 which has two branch pipes 10 leading into the upper end of the digester 25 at diametrically opposite points like the inlet pipes 2 at the bottom. In the top of the digester is a man-hole 11 through which the straw B can be loaded into the digester, and at the bottom is a similar man-hole 12 30 through which the stock can be removed after it has been subjected to the treatment about to be described. When the apparatus is in use these man-holes are tightly sealed by means of covers or man-hole plates 13 so 35 as to be steam tight and water tight.

When the digester has been filled up with straw, warm water is introduced into the bottom of the digester through the pipe 3, while the valve 14 in the outlet pipe 9 is 40 left open. The warm water is obtained by opening the valve 7 in the water supply pipe 4 and partly opening the valve 8 in the steam pipe 5, whereby the steam will heat the water in its passage to the digester. 45 When the water has risen nearly to the top of the digester, leaving an air space of from 12 to 18 inches above it the valve 14 at the top is closed and the supply of water is shut off by closing the valve 7 while the 50 steam valve 8 is opened to turn the live steam full on. I prefer to heat the water before it enters the digester; otherwise the steam would condense and the water of condensation might be so much as to fill the 55 digester and block the passage of the steam.

The steam entering the digester will heat the water therein to the boiling point, and the steam and hot water will pass up and circulate through the mass of straw and cook 60 the same so as to soften and loosen up the coloring matter and gummy constituents thereof. This cooking should continue to about three hours. Then the valve 8 in the steam supply pipe is partly shut and water 65 turned on by opening the valve 7, the water

being heated by the steam coming through the partly open valve 8. The valve in the pipe 9 at the top is then partly opened so as to let off steam and allow a circulation of the water and steam through the digester 70 while still maintaining a pressure therein. The brown liquor containing the gummy constituents, dirt, and colored matter will thus be forced out through the pipe 9 at the top by the water and steam entering at 75 the bottom, while the contents of the digester are still under pressure.

This circulation is allowed to continue from three to twelve hours according to the color and quality of the stock that is desired. The longer the circulation is continued, the more completely will the gums and coloring matter be washed or separated out. If the product desired is only "half-stock" so-called, wherein the fibers are only 85 partly separated and degummed, the circulation need not be continued for more than the shorter period above named, but to reduce it to full paper stock the circulation must be continued longer.

90 When the circulation has been carried far enough the valve 8 in the steam pipe is closed and the valve 7 opened to allow cold water to be forced into the bottom of the digester. This water will rise up through 95 the mass and force the remainder of the hot gummy colored liquor out at the top and wash the stock. It is important that this water should be cool, so that it will not mix with the warm gummy liquor in the digester, 100 but will force this liquor bodily up and out through the outlet pipe 9. As soon as the digester begins to get cool at the top the liquor will run clear showing that the gums and the coloring matter which has been freed 105 have been very completely forced out. The mass is then ready to be removed from the digester through the man hole 12 at the bottom.

110 When the circulation has been continued long enough to form full paper stock the fibrous mass is so clean and free from gums and coloring matter and from the brown gummy liquor that it does not need any further washing, and the fibers are so separated and free from lumps and hard or unseparated particles that the mass does not need beating in the usual beating machine, but is ready for use as paper stock in the paper making process, and the product is of 115 uniform texture and will not become lumpy when formed, whereby the paper made from it will not be hard and brittle like the old fashioned butcher's wrapping paper, but will be soft, clear and tough.

120 By the present process therefore I am enabled to effect a very complete removal of the coloring matters and gummy constituents of the straw without the use of chemicals and without any loss of stock or breaking 125

up of the long fibres which are so desirable in giving strength to the paper. While the process is particularly intended for the treatment of cereal straw, it is equally applicable to any other kind of straw or fibrous material having gums or coloring matter to be removed.

By the term "pressure" as herein used I mean a pressure greater than atmospheric pressure.

When removed from the digester in the condition of "half-stock," that is before all the fibers have been degummed and separated, the product will form an excellent heat insulating product because of its light weight and spongy texture due largely to the very complete removal of the gummy liquor, and because of the intimate admixture and intertanglement of the finer mass of more or less completely degummed and separated fibers with the coarser unseparated particles, this admixture being possible because the treatment has been such as not to destroy these fine fibers.

I claim:

1. The herein described process of making paper stock from straw containing a gummy constituent which consists in cooking the straw in water and under pressure to loosen up the gummy constituent, and then forcing out the gummy liquor formed in cooking while the same is still warm and under pressure.

2. The herein described process of making paper stock from straw containing a gummy constituent which consists in cooking the straw until the gummy constituent has become loosened up, and then forcing cold water through the cooked mass while the

same is under pressure and still warm, 40 whereby to drive off the gummy liquor.

3. The herein described process of making paper stock from straw containing a gummy constituent which consists in cooking the straw in water under pressure to loosen up 45 the gummy constituent, and then forcing cold water through the cooked mass while the same is still heated and under pressure, whereby to drive off the gummy liquor.

4. The herein described process of making 50 paper stock from straw containing a gummy constituent which consists in first cooking the straw in water and under pressure to loosen up the gummy constituent, then forcing warm water through the mass while the 55 same is under pressure to drive off the gummy matter thus loosened up and then forcing cold water through the mass while same is under pressure and still warm, whereby to wash out the gummy liquor 60 without allowing it to become mixed with said cold water.

5. A fibrous product of the herein described process formed by first cooking cereal straw in water and under pressure to 65 loosen up the gummy constituents thereof, then forcing warm water through the mass while the same is still warm and under pressure to wash out the gummy matter thus loosened up, and then driving off the gummy 70 liquor while the same is still warm, substantially as described.

In testimony whereof I affix my signature in presence of two witnesses.

JAMES E. LAPPEN.

Witnesses:

LL. SWANSON,  
ARTHUR P. LOTHROP.